# EUROPEAN PATENT SPECIFICATION

(11) **EP 1 195 642 B1**
(45) Date of publication and mention of the grant of the patent: **25.02.2004**
(21) Application number: 01000462.0
(22) Date of filing: 14.09.2001
(51) Int. Cl.: G03C 1/09, G03C 1/005, G03C 5/17, G01T 1/08

(54) **Silver halide photographic material and image-forming system in direct X-ray imaging applications**
Photographisches Silberhalogenidmaterial und Bilderzeugungssystem für die Verwendung in der direkten radiographischen Bilderzeugung
Matériau photographique à l'halogénure d'argent et système de formation d'images pour des applications de production d' images radiographiques directes

(30) Priority: 04.10.2000 EP 00203438
(43) Date of publication of application: 10.04.2002
(73) Proprietor: AGFA-GEVAERT, 2640 Mortsel (BE)
(72) Inventor: Van den Zegel, Marc c/o Agfa-Gevaert, 2640 Mortsel (BE); De Vester, Marleen c/o Agfa Gevaert, 2640 Mortsel (BE)

(56) References cited:
- EP-A- 0 757 286
- GB-A- 758 475
- US-A- 5 397 692
- US-A- 5 766 837

## Description

The present invention relates to a direct X-ray sensitive black-and-white silver halide photographic material having radiation sensitive silver halide emulsion layers comprising negative image type tabular emulsion crystals, a method of image formation in the field of direct X-ray radiography and a direct X-ray system suitable for use in non-destructive testing applications and personal monitoring.

### BACKGROUND OF THE INVENTION

In industrial radiography non-destructive techniques for testing and analyzing defects in components such as glass, paper, wood or metal parts, etc. are well-known. This technique is e.g. widely used in aeronautics, the nuclear industry or the petroleum industry since it makes it possible to detect welding defects or defects in the texture of materials in aircraft components, nuclear reactors or pipelines. This technique consists of exposing a component to be analyzed to an ionizing radiation, in general X- or gamma rays having an energy between 10.000 and 15.000 kVp, either by direct X-ray radiography or by means of an intensifying screen. It is therefore necessary with this technique to use specific radiographic elements which are highly sensitive to this ionizing radiation. The major part of the ionizing radiation however passes through the silver halide grains without being absorbed and only a very small part of the incident radiation (less than 1%) is really absorbed and contributes to the formation of a developable latent image.

In order to really achieve high film sensitivity, also called "speed", which is an indispensible asset especially for directröntgen applications, efficient absorption of the exposure radiation is a prime condition. It has been shown empirically that for X-rays the mass absorption coefficient is proportional to a power of the atomic number Z as has been described in the "Encyclopaedic Dictionary of Physics" vol. 7, p. 787, eq. 10, Ed. J.Thewlis, Pergamon Press, Oxford 1957. This strongly favours the use of iodide(Z=54), more than bromide (Z=35) and further more than chloride (Z=17). As a consequence silver bromo(chloro)iodide crystals have preferably been used hitherto. Absorption of the ionizing radiation can further be enhanced by increasing the silver content and/or the thickness of the emulsion layers. Moreover it is common knowledge to provide double-side coated materials in favour of absorption of high energy radiation.

Cubic silver bromoiodide grains have until now preferably been used in non-destructive testing applications for the reason set out above, preferably coated in high amounts of more than 25 g/m2, expressed as equivalent amounts of silver nitrate, particularly when a higher speed is envisaged, as for those materials having grains with an average equivalent crystal diameter of at least 0.4 µm or an average equivalent volume of at least 0.034 µm³. Lowering of coated amounts of silver thus results in a reduction of speed (sensitivity) for direct-Röngten rays and further leads to a lowering in contrast, which may be in favour of image quality (especially graininess) as desired for some well-designed applications, but makes maximum density decrease to an unacceptable level. When in such case use can only be made of radiation sources for X-rays having a lower energy output (exposure energies of about 100 kVp instead of the normally used 220 kVp) besides undesired higher contrasts a reduced speed can be expected. Although said reduced speed can be compensated in industrial radiographic exposure techniques by application of intensifying screens in contact with industrial non-destructive test film materials, thereby taking profit of the combined effect of direct-Röntgen exposure and exposure by light emitted from light-emitting or luminescent phosphors present in the intensifying screens (making that the system as a whole is not a direct X-ray system), the problem of too high contrasts remains in that case.

A suitable solution therefor has been presented in EP-A 0 890 875 and the corresponding US-A 6,030,757 wherein a multilayer arrangement has been disclosed for a material suitable for e.g. concrete testing and wherein use was made, besides the well-known cubic grain emulsions, from tabular grain emulsions.

Said tabular grains, known for practical applications in photography since the eighties, have however already been proposed in EP-A 0 757 286 and the corresponding US-A 5,965,337 as being effectively suitable for use in industrial non-destructive testing applications, moreover providing an improved speed. An indication of the applicability of tabular grain emulsions was already given before in dental X-ray applications in EP-A 0 653 670 and the corresponding US-A 5,370,977. Although claiming applicability of tabular grains having improved speed in an industrial radiographic element designed to be exposed to X-rays or gamma-rays having an energy greater than or equal to 10 kV, it has been derived from our experiments that when exposing such a material to irradiation, generated from a Co-60 source, in applications such as concrete search, speed is insufficient and that materials having tabular grain emulsions as presented therein are not suitable for use in such specific industrial non-destructive testing applications.

### OBJECTS OF THE INVENTION

It has been an object of the present invention to provide silver halide photographic film materials for direct X-ray applications as e.g. industrial non-destructive testing applications and personal monitoring, offering high speed after processing of said materials after having been exposed to high-energy radiation exposure by X-ray of gamma-ray sources, as e.g. from a Co-60 source, and to provide a system in order to get images having high image quality.

Other objects will become apparent from the description hereinafter.

### SUMMARY OF THE INVENTION

The objects of the present invention have been attained by providing a direct X-ray radiographic element comprised of a support covered on at least one of its major faces with a tabular grain emulsion layer free from spectrally sensitizing dyes, in which at least 50 percent of total grain projected area is accounted for by silver bromoiodide tabular grains having silver iodide in an amount of at most 1 mole % based on silver, having an average volume between 0.05 and 2 µm³ and an average aspect ratio between 5 and 25, wherein a silver content per coated side, expressed as an equivalent amount of silver nitrate, is between 5 and 25 g/m², characterized in that said tabular grain emulsion(s) have selenium in an amount of 0.5 to 20 µmole per mole of silver nitrate (as having been subjected to chemical sensitization in the presence of a compound providing selenium).

Further a system for direct X-ray radiography has been provided, said system being comprised of (1) a direct X-ray radiographic element according to the present invention and (2) disposed on opposite sides of the radiographic element, two intensifying screens designed to emit electrons when exposed to X or gamma rays with an energy greater than or equal to 10 kVp.

Moreover a method for forming a radiographic image has been provided, said method comprising the steps of
(1) exposing a system according to the present invention, to X- or γ-rays with an energy greater than or equal to 10 kVp or, in a particular embodiment, with the energy of a Co-60 source in order to form a latent image and (2) developing said latent image.

Specific features for preferred embodiments of the invention are set out in the dependent claims.

Further advantages and embodiments of the present invention will become apparent from the following description.

### DETAILED DESCRIPTION OF THE INVENTION

It has quite unexpectedly been found that, although chemical ripening of silver halide emulsion crystals with a compound providing selenium in the chemical sensitization step is known for years, that a remarkable, and completely unexpected, speed increase is attained in industrial non-destructive testing materials when exposed to radiation from high energy sources like Cobalt-60, further called "Co-60" in amounts of selenium as prescribed in the summary of the invention and in the claims. As is well-known Co-60 emits two high energy spectrum lines of radiation (1.1 and 1.3MeV) and it is only this radiation, attenuated during transmission through the specimen, which forms the images of flaws in the specimen. There is no primary lower energy radiation from the source. Some of this radiation absorbed in the specimen is re-emitted as Compton scattered radiation of lower energy and as such reaches the film, but it only degrades the image contrast, and any intensifying screen which accentuates this scattered radiation enhances this image degradation. Two conclusions are therefore evident:
1. The radiation spectrum with cobalt-60 gamma-rays is quite unlike that from any X-ray tube.
2. A front intensifying screen having moderate thickness in order to avoid a negative influence on image sharpness during irradiation is desirable, which will preferentially absorb some of the scattered radiation, and not produce much intensification from this scattered radiation. In practice in the system according to the present invention screen sheets selected from the group of lead, lead oxide, copper and steel are preferred, wherein said screens appear to satisfy the second requirement, but other materials used with a metal filter may be used. These intensifying screens, not emitting light as luminescent phosphor screens used in "indirect" X-ray radiography, enable the proportion of ionizing radiations absorbed by the silver halide grains to be increased and make part of the direct X-ray system as such. So the X-rays interact with the intensifying screen, producing electrons in all directions and some of these electrons will be absorbed by the silver halide grains in the emulsion layer in order to form latent image sites. By increasing the number of electrons emitted in the direction of the grains, the quantity of electrons absorbed by the grains is increased. The thickness of these screens is between 0.025 mm and 0.5 mm, depending on the type of ionizing radiation used. In a preferred embodiment the element according to the present invention the sheet film is packed in a daylight packaging, e.g. the packaging known as Pb Vacupac, Pb ETE (Edge to Edge) and DW ETE (Edge to Edge), known as trademark products from Agfa-Gevaert N.V., Mortsel, Belgium. The Pb Vacupac is completely light-tight, air-tight and moisture-proof. It provides optimal image quality and is easy to use. Just as the STRUCTURIX® X-ray films with Pb screens are vacuum-packed in a synthetic foil that ensures that Vacupac® can be used under extremely dirty and damp conditions, ideal for applications with energies higher than 100 kV. The vacuum ensures that contact between the film and the lead screens is perfect, guaranteeing optimal image definition. The easy-to-use wrapper allows rapid positioning and can be opened in one movement.

What is sometimes referred to as "a plastic envelope with prepacked lead screens" happens to be a very "HighTech, High-Chem" complex. The flexible vacuum packaged receptor is composed of 21 layers, each layer being the result of research and development with regard to the permanent striving for a better image quality. The extrusion technology of polyester base suitable for photographic applications (materials); the emulsion layers, coated on this base, are composite matrixes integrating silver halide emulsion crystals coated therein as semiconductor light receptors; screen technology (type of paper and glue, not least the lead alloy combining photon-absorption, electron emission with mechanical properties) providing enhanced contrast and speed; outer wrapping with flexible mirrors consisting of vacuum deposited aluminium on thermoplasts and reinforced and protected with polymers. Such packaging has been disclosed in the US-A's 4,586,311 and 5,413,901.

According to the present invention a direct X-ray radiographic element is provided, said element or material being comprised of a support covered on at least one of its major faces with a tabular grain emulsion layer free from spectrally sensitizing dyes, in which at least 50 percent of total grain projected area is accounted for by silver bromo iodide tabular grains having silver iodide in an amount of at most 1 mole % based on silver, having an average volume between having an average aspect ratio between 5 and 25, and having a average volume between 0.05 and 2 µm³ and wherein a silver content per coated side, expressed as an equivalent amount of silver nitrate, is between 5 and 25 g/m², characterized in that said tabular grain emulsion(s) has or have selenium in an amount of 0.5 to 20 µmole per mole of silver nitrate.

In one embodiment said direct X-ray element comprises a support, at least one silver halide emulsion layer and a non-light sensitive hydrophilic colloidal layer, wherein the silver halide emulsion layer comprises a selenium compound represented by formula (1) : wherein:
- Q represents R¹SO₂ or R²R³P=X;
- each of R¹, R² and R³ the same or different represents OR⁴, NR⁵R⁶, SR⁷, SeR⁸ or an alkyl group, an aryl group or a heteroaryl group;
- X represents O, S or Se;
- each of R⁴, R⁵, R⁶, R⁷ and R⁸ the same or different represents hydrogen, an alkyl group, an aryl group or a heteroaryl group, or R⁵ and R⁶ together represents the atoms necessary to form a N-containing ring.

A method in order to prepare a photosensitive direct X-ray element or material as described hereinbefore comprises the step of chemically sensitizing at least one of the silver halide emulsions by means of a selenium compound according to formula (1) and, preferably, in the presence of a silver halide solvent at a pH-value situated between 3 and 10, a pAg-value between 6 and 11 and a temperature in the range of from 40°C up to 95 °C.

A preferred group of compounds which are suitable for use in the chemical sensitization of at least one emulsion, to be coated in the photosensitive element for direct X-ray radiology as applied herein is represented by formula (2): where R⁹ is restricted to an alkyl group, an aryl group or a heteroaryl group.

Another preferred group of compounds included by the general formula (1) of this invention with respect to the selenium compound is described by formula (3): wherein:
- x represents O, S or Se;
- R¹⁰ represents an alkyl group, an aryl group, a heteroaryl group or an alkoxy group.

Specific examples of selenium compounds which can be used in the photographic material of the present invention include the following diselenium disulphonates:

Other specific examples of selenium compounds for use according to the present invention are the following phosphoric-diselenides (see the structures P-I to P-XI):

The compounds represented by general formula (1) can be synthesized according to known methods or as has been described in US-A 5,910,402.
It is recommended to chemically sensitize said silver halide emulsion grains with one or more unstable selenium compound(s).
Specific well-known examples of unstable selenium sensitizers are isoselenocyanates (e.g., aliphatic isoselencyanates such as allylisoselenocyanate), selenoureas, selenoketones, selenoamides, selenocarboxylic acids (e.g. 2-selenopropionic acid, and 2-selenobutyric acid) selenoesters, diacylselenides (e.g. bis(3-chloro-2,6-dimethoxybenzoyl)selenide), selenophosphates, phosphineselenides as triphenylphosphorselenide and colloidal elemental selenium.

In another embodiment of the present invention unstable selenium compounds, generating silver selenide in an emulsion comprising said grains at a temperature of from 45°C up to 70°C and at an electrical potential difference between a silver electrode and a saturated silver/silver chloride reference electrode of from 100 up to 200 mV are particularly preferred. In the well-defined circumstances given hereinbefore it is possible to reach the required speed at low fog levels and with the desired sensitometric stability in the image-forming system of the present invention.

In still another embodiment of the present invention, for the emulsion grains used in the photosensitive direct X-ray element and in the image-forming system according to the present invention (called "primitive" or "unripened" as long as no chemical sensitizer(s) is(are) added after precipitation and redispersion of said grains), addition of selenium compounds generating silver selenide in the prescribed circumstances is required. Such selenium compounds are preferably compounds selected from the group consisting of substituted selenoureum, substituted triphenylphosphine selenide and substituted and unsubstituted triphenylorthophosphate selenide.

Specific examples of those groups of compounds have been given hereinafter (see the formulae I to VII), without however being limited thereto:
- triphenyl-tricarboxylic acid substituted phosphine selenide
- triphenyl-dicarboxylic acid substituted phosphine selenide
- triphenyl-(mono)carboxylic acid substituted phosphine selenide
- triphenyl-sulphonic acid substituted phosphine selenide
- triphenylorthophosphate selenide

The emulsion grains suitable for use in the direct X-ray element according to the present invention should optionally further be chemically ripened with one or more sulphur and/or gold compounds.
Useful patent literature with respect to the use of selenium sensitizers and to the chemical ripening process of silver halide emulsion grains, suitable for use in the context of the present invention can e.g. be found in EP-A's 0 443 453, 0 454 069, 0 488 029, 0 638 840, 0 661 589, 0 638 840 and 0 809 136, and in US-A's 5,114,838; 5,028,522; 5,112,733; 5,158,892; 5,306,613; 5,364,754; 5,389,511; 5,397,692; 5,518,873; 5,547,829; 5,573,901; 5,578,435; 5,654,134; 5,766,837; 5,807,662; 5,853,972; 5,888,717 and 5,965,343. Commonly said selenium sensitizers are used together with other sensitizers as at least gold and optionally sulphur and/or even tellurium.

Especially useful labile compounds providing sulphur are compounds selected from the group consisting of tetramethylthiodithioacetic acid diamide, dimethylamino-dithiomercaptane, thiosulphate and thiosulphonate compounds. Other useful compounds are those as described e.g. in "Chimie et Physique Photographique" by P. Glafkides, in "Photographic Emulsion Chemistry" by G.F. Duffin, in "Making and Coating Photographic Emulsion" by V.L. Zelikman et al, and in "Die Grundlagen der Photographischen Prozesse mit Silberhalogeniden" edited by H. Frieser and published by Akademische Verlagsgesellschaft (1968).

As described in said literature chemical sensitization can be carried out by effecting the ripening in the presence of small amounts of compounds containing sulphur as e.g. thiosulphate, thiocyanate, thioureas; sulphites, mercapto compounds, rhodamines wherein combinations of gold-sulphur ripeners together with the required selenium sensitizers are the most preferred.

Addition of tellurium compounds as e.g. tellurosulphate, tellurocyanate, telluroureas in very small amounts is thereby however not excluded. Further reductors as e.g. tin compounds as described in GB-A 789,823, amines, hydrazine derivatives, formamidine-sulphinic acids, and silane compounds may be used, although care should be taken in order to prevent the emulsion from fog formation in an uncontrollable way.

According to the present invention amounts of selenium compounds in the said tabular grain emulsion(s) of the industrial radiographic elements are in the range from 1 x 10⁻⁵ to 5 x 10⁻⁷ moles (0.5 to 10 µmole) per mole of silver nitrate. Normal amounts of gold compounds (as gold chloride or gold thiocyanate) are in the range from 1 x 10⁻⁵ to 2.5 x 10⁻⁵ moles per mole of silver nitrate. Preferred amounts of gold salts to be added of at least 0.010 mmole per mole of silver should at least be accompanied by a sulfite salt, to be added in an amount of at least 0.05 mmole per mole of silver.

As has already been suggested hereinbefore the use of reducing agents in the chemical ripening of silver halide emulsion crystals is not excluded either as depending upon the circumstances it may be recommended to use small amounts in order to counterbalance the restraining actions from fog-restrainers or stabilizers as e.g. substituted heterocyclic mercapto-compounds described in US-A 5,242,791. Silver solvents may have a regulating role therein as e.g. those comprising thiocyanate ions.

It is a common method to add chemical sensitizers after redispersion. As, according to a preferred embodiment, the element of the present invention has emulsions, free of spectrally sensitizing dyes, the moment of addition of the chemical sensitizing agents is less critical as otherwise addition of chemical sensitizers as so-called "site-directors" during and/or after spectral sensitization would be preferred.

Before starting chemical sensitization the surface of the tabular silver halide grains may be treated with slightly oxidizing compounds as e.g. toluene thiosulphonic acid and/or corresponding salts thereof in order to reduce small silver specks to grow to fog centers in an uncontrolled manner.

The introduction of the chemical selenium sensitizer can be done in various ways before starting the chemical sensitization procedure. Selenium sensitizers which are more or less water soluble can be added to the dispersion of silver halide crystals as an aqueous solution if desired mixed up with a water soluble organic solvent. Selenium sensitizers which are not water-soluble can be introduced after dissolving the compound in a water soluble organic solvent which is normally used for the introduction of water insoluble products in a photographic silver halide emulsion. An alternative way for the introduction of an insoluble chemical chalcogenic sensitizer is using an 'oil-in-water' dispersion or, if desired, a dispersion as disclosed in EP-A 0 703 492. In the last named patent application the said compound is therefore added to the silver halide emulsion before chemical sensitization in form of a solid partical dispersion in water.

The chemical sensitization with selenium compounds providing the tabular grains used in the preferred radiographic non-destructive material or element of the present invention with selenium in an amount as claimed, is preferably carried out in the presence of a silver halide solvent like e.g. a thiocyanate salt. This can be added as a sodium, a potassium or preferably as an ammonium salt, without however being limited thereto. The thiocyanate salt can be added before, during or after the addition of said compound used in the invention and before, during or after the addition of any other chemical sensitizer which can be used together with the said selenium sensitizer. The amount of the thiocyanate which is present together with the said chemical sensitizer is limited between 10⁻⁶ and 10⁻¹ mole per mole of silver halide and preferably between 10⁻⁵ and 10⁻² mole per mole of silver halide.
The selenium compounds used in the element of the present invention can be used in combination with other known selenium sensitizers. The selenium sensitization itself can be carried out in the presence of a sulphur compound and, if desired, in the presence of a noble metal (e.g. gold), whether or not in combination with reduction sensitizer.

As already set forth hereinbefore a tabular grain emulsion in which at least 50 percent of total grain projected area is accounted for by silver bromo iodide tabular grains having an iodide content of at most 1 mole %, based on silver, having an average aspect ratio between 5 and 25, and having a volume between 0.05 and 2 µm³ is desired. When the direct X-ray radiographic element is intended to be exposed to high-energy radiation (above 500 kVp), the volume of the tabular grains is preferably greater than 0.06 µm³.
Further according to the present invention said element is coated with photosensitive emulsion crystals so that a silver content per coated side, expressed as an equivalent amount of silver nitrate, is between 5 and 25 g/m².

Tabular silver halide grains having a {111} crystal habit have been promoted since 1982 as being applicable in photographic materials for practical use and are defined as crystals possessing two parallel faces with a ratio between the diameter of a circle having the same area as these faces (the so-called equivalent circular diameter or E.C.D.), and the thickness, being the distance between the two major faces (said thickness being measured from a carbon replica of the grain, shadowed under an angle of 30° and measuring the length of the shadow), equal to at least 2. In the present invention {111} tabular silver bromo(chloro)iodide grains have aspect ratios of from 5 to 20 and tabularities, defined as the ratio of aspect ratio and thickness or between E.C.D. and thickness square, of from 20 to 200.

Incorporation of iodide ions in the preferred tabular silver bromoiodide crystals may further be provided by using aqueous solutions of inorganic salts thereof as e.g. potassium iodide, sodium iodide or ammonium iodide. Iodide ions can however also be provided by organic compounds releasing iodide ions as has e.g. been described in EP-A's 0 561 415, 0 563 701, 0 563 708, 0 649 052 and 0 651 284 and in WO 96/13759. Especially in order to obtain a more homogeneous iodide distribution over the crystal volume in the crystal lattice and over the whole crystal distribution, iodide ions provided by organic agents releasing iodide ions are preferred such as mono iodide acetic acid, mono iodide propionic acid, mono iodide ethanol and even hydrogels containing iodide ions, capable to generate iodide ions. Generation of iodide ions is triggered by changing the pH value in the reaction vessel during or, preferably, after addition of the said organic agent releasing iodide ions. Opposite to the addition of potassium iodide as a source of iodide ions the said organic compounds releasing iodide ions are leading to a more homogeneous iodide ion distribution over the different tabular crystals, thus avoiding undefined heterogeneities and irreproducibilities. Another method of triggering generation of iodide ions is performed by addition of sulphite ions to the reaction vessel. Combinations of inorganic and organic agents providing iodide ions may also be useful. Alternatively very fine silver iodide grains, having a grain diameter of about 0.05 µm may be added as a source of iodide ions (also in favour of uniformity of silver iodide distribution over the tabular grains as disclosed e.g. in US-A 5,955,253), and even addition of KI₃ is not excluded (see e.g. US-A 6,033,842). Although normally added during the precipitation step(s) said iodide ions can be added (in small amounts) during the chemical sensitization step (even in form of those small silver iodide grains as has e.g. been described in US-A 5,411,849. The presence of iodide ions stabilizes the (111)-crystal faces. Although preferred with respect to intrinsic sensitivity or speed, it is recommended to limit average iodide concentrations in the range from 0.1 mole % to 1.0 mole %, based on the total silver amount as higher concentrations retard development and lead to unsatisfactory sensitivities. Moreover the velocity of fixation can be disturbed in that case and as a consequence residual coloration may be unavoidable.

Grain size distributions of the preferred silver bromoiodide crystals over the light-sensitive emulsion are homogeneous or monodisperse by controlling the precipitation methods used. Metal ions or metal ion complexes, also called dopants, commonly added in low amounts to the silver bromoiodide crystals in whatever a stage of the preparation, generally have little influence on crystal distributions in the emulsions but may be added to cause advantageous effects with respect to reciprocity, pressure sensitization, as has been described e.g. in US-A 5,362,619; wherein fine AgI crystals have been added in the precipitation step.

Therefore it is very important to carefully control pAg, temperature, dilution of the reaction vessel, presence of growth restrainers or growth accelerators, addition rate of added aqueous soluble silver salt and halide solutions during different precipitation steps (especially during the nucleation step during which e.g. less than 10 % of the total amount of silver salt available is consumed and further during the at least one growth step during which at least 90 % of the said silver salt is consumed), way of mixing and mixing or stirring rate in the reaction vessel during the different precipitation steps leads to homogeneous crystal size distributions having variation coefficients (defined as ratio between standard deviation and average diameter) of not more than 0.10 to 0.20 instead of the normally occurring variation coefficients between 0.20 and 0.30. Depending on the precipitation conditions more heterogeneous distributions can be obtained and may even be more advantageous e.g. from the point of view of exposure latitude but in order to obtain the same effect of e.g. an increasing exposure latitude is reached by making mixtures of different homogeneous emulsions having very low variation coefficients e.g. in the range from 0.05 to 0.15. This may lead to even more advantageous sensitometric characteristics (e.g. increased contrast) or image quality (e.g. granularity and/or sharpness) as has been illustrated e.g. in US-A 4,446,228 and in EP-A 0 555 897.

For practical use thin tabular grains accounting for at least 50 % of the total projective surface area of all grains, more preferred for at least 70 % and still more preferred for at least 90 %, are present.

The composition of the halide can change in the crystal in a continous or discontinous way. Emulsions containing crystals composed of various sections with different halide compositions are used for several photographic applications. So a structure with a difference in halide composition between the center and the rest of the crystal (what is called 'core-shell'-emulsion) or with more than two crystal parts differing in halide composition (called a 'band'-emulsion) may occur. The changes in halide composition can be realized by direct precipitation or in an indirect way by conversion where fine silver halide grains of a certain halide composition are dissolved in the presence of the so-called host grains forming a 'shell' or 'band' on the given grain.

As already set forth noble metal sensitization of a salt of a noble metal (e.g., gold, iridium, palladium, platinum) is applied, wherein gold salts are preferably used as noble metal sensitizer. Examples of gold sensitizers which are often used include chloroauric acid, goldsulfide, chloroaurate salts, aurithiocyanate and gold selenide. The amount of the noble metal sensitizer can vary between 10⁻⁸ and 10⁻² mole per mole silver halide.
Sulfur sensitization can be carried out with sulphur compounds like thiosulphates, thioureas, rhodamines. The sulphur sensitizer can also be used in an amount of about 10⁻⁸ to 10⁻² mole per mole silver halide. Tellurium sensitization can even be optionally applied, as e.g. disclosed in US-A's 5,273,874; 5,215,880; 5,561,033; 5,393,655; 5,547,829; 5,888,717; 5,677,120; in EP-A's 0 572 663 and 1 070 986, in GB-A 2,316,184, and in DE 19924669.

In reduction sensitization a reducing compound is used like thiourea dioxide, hydrazine derivatives, sulphinic acid, polyamine compounds, stannous chloride, borane compounds, reductones like ascorbic acid. Reduction sensitization can also be carried out at a low pAg or a high pH or at both and if desired at elevated temperature. This kind of sensitization is refered to 'silver ripening'. More information can be found in Research Disclosure, Vol 307,307105 and in P.Glafkides "Chimie et Physique Photographiques", P.Montel - Paris, 5^{th} Ed., 1987.

Preparation of a direct X-ray photosensitive element according to the present invention essentially comprises the step of chemically sensitizing at least one silver halide emulsion in the presence of the selenium compound in preferred amounts as disclosed hereinbefore. The chemical sensitization step is preferably carried out under conditions of pAg in the range of 6 till 11 but preferably between 7 and 10, in conditions of pH in the range of 3 to 10, preferably 4 to 8.5, while the temperature is in the range between 40 to 95°C, preferably between 45 and 85°C. There are no particular limitations to any of these conditions.

The silver halide emulsion can be prepared in various ways by conventional methods. These always start with a nucleation phase followed by a grain growth phase. In this last phase of the emulsion preparation reactants are added to the reaction vessel in the form of solutions of silver and halide salts or in the form of preformed silver halide nuclei or fine grains which easily dissolve in the precipitation medium.

Individual reactants can be added through surface or subsurface delivery tubes by hydrostatic pressure or by an automatic delivery system for maintaining the control of pH and/or pAg in the reaction vessel and of the rate of the reactant solutions introduced in it. The reactant solutions or dispersions can be added at a constant rate or a constantly increasing, decreasing or fluctuating rate, if desired in combination with stepwise delivery procedures. More details about the possible ways in making a silver halide emulsion which can principally be used in this invention are summarized in Res.Discl.,38957 (sept. 1996) section I-C.

Besides individual reactants necessary to form silver halide crystals, additional chemical metal salts can be added for occlusion in the crystal lattice. Such compound is replacing an appropiate of silver and halide ions in the silver halide lattice. These products or so-called dopants can be distinguished from the metal complexes which are added just before coating as an additive by EPR- or ENDOR-technique. These dopants can be used to modify the crystal structure or the crystal properties and can therefore be employed to influence many photographical properties like sensitivity, reciprocity failure, gradation, pressure sensitivity, fog, stability. When coordination complexes or even oligomeric coordination complexes are used the different ligands bound at the central metal ion can be occluded in the crystal lattice too and in this way influence the photographic properties of the silver halide materials as well. Dopants which are introduced in emulsions used in the present invention are those which can act as a permanent or as a non-permanent electron trap. The doping procedure itself can normally be executed at any stage during the grain growth phase of the emulsion preparation. It is important to know that the dopants can also be added in an indirect way by the addition of a dispersion containing very fine soluble silver halide grains or nuclei comprising the dopant. More additional information about the introduction and the use of dopants in the emulsion crystals can be found in Research Disclosure, 38957 (sept. 1996), section I-D. Doping agents, generally in small quantities, such as rhodium, indium, osmium, iridium and ruthenium ions can be added and incorporated in a way as has further been disclosed in e.g. in US-A's 5,306,613; 5, 399,476; in EP-A's 0 933 670, 0 933 671, 1 045 282 and in EP-Application No. 99201625, filed May 25, 1999. Incorporation of organic hole trapping dopants, e.g. making use of formic acid, rongalites, can also be applied as described in EP-A 0 922 994.

As is well-known gelatin is normally used as protective colloid for the silver halide emulsion crystals during precipitation. The preparation of conventional lime-treated or acid treated gelatin has been described in e.g. "The Science and Technology of Gelatin", edited by A.G. Ward and A. Courts, Academic Press 1977, page 295 and next pages. The gelatin can also be enzyme-treated as described in Bull. Soc. Sci. Phot. Japan, N° 16, page 30 (1966). A preparation method of tabular grain emulsions wherein in the grain growth process use is made of gelatin derivatives with chemically modified NH₂-groups and wherein said gelatin has a specific methionine content has been described in e.g. EP-A 0 697 618. Gelatin may, however, be replaced in part or integrally by synthetic, semi-synthetic, or natural polymers. Synthetic substitutes for gelatin are e.g. polyvinyl alcohol, poly-N-vinyl pyrrolidone, polyvinyl imidazole, polyvinyl pyrazole, polyacrylamide, polyacrylic acid, and derivatives thereof, in particular copolymers thereof. Natural substitutes for gelatin are e.g. other proteins such as zein, albumin and casein, cellulose, saccharides, starch, and alginates. In general, the semi-synthetic substitutes for gelatin are modified natural products e.g. gelatin derivatives obtained by conversion of gelatin with alkylating or.acylating agents, by grafting of polymerizable monomers on gelatin or prehardened gelatins with blocked functional groups as a consequence of this prehardening treatment, cellulose derivatives such as hydroxyalkyl cellulose, carboxymethyl cellulose, phthaloyl cellulose, and cellulose sulphates and even even cationic starch, whether or not in oxidized form. Further synthetic high molecular compounds described in JP-B-52-16365, Journal of The Society of Photographic Science and Technology of Japan, Vol. 29(1), 17, 22(1966), ibid., Vol. 30(1), 10, 19(1967), ibid., Vol. 30(2), 17(1967), and ibid., Vol. 33(3),24(1967) may be used as a dispersion medium. Also the crystal habit restraining agent described in EP-A 0 534 395 may be used.
Part of gelatin may further be replaced with a synthetic or natural high-molecular material.
An interesting substitute for gelatin may be silica as has been described in the published EP-A's 0 392 092, 0 517 961, 0 528 476, 0 649 051, 0 677 773 and 0 704 749. As has been set forth in EP-A 0 528 476 a method of preparing a silver halide light-sensitive photographic material incorporating layers of silver halide precipitated in colloidal silica serving as a protective colloid is given. In this document the silver halides are prepared in colloidal silica, leading to emulsion crystals that are stable at the end of the precipitation, without however having a predictable mean crystal diameter and crystal size distribution.
For the precipitation processes wherein suitable silica sols are required as colloidal binder, said silica sols are commercially available such as the "Syton" silica sols (a trademarked product of Monsanto Inorganic Chemicals Div.), the "Ludex" silica sols (a trademarked product of du Pont de Nemours & Co., Inc.), the "Nalco" and "Nalcoag" silica sols (trademarked products of Nalco Chemical Co), the "Snowtex" silica sols of Nissan Kagaku K.K. and the "Kieselsol, Types 100, 200, 300, 500 and 600" (trademarked products of Bayer AG). Particle sizes of the silica sol particles are in the range from 3 nm to 30 µm. The smaller particles in the range from 3 nm to 0.3 µm, and still more preferable from 3 nm up to 7 nm are preferred as the covering degree that can be achieved will be higher and as the protective action of the colloidal silica will be more effective.

At the end of the precipitation, following all possible physical ripening steps, the emulsion mixture is normally cooled to about 40°C, before or after adding a flocculate being a polymeric compound as e.g. polystyrene sulphonic acid, providing as a anionic polymer a behaviour depending on pH. Under carefully controlled conditions of addition and stirring rate the pH of the said dispersing medium is adjusted with an acid to a value in order to get a qualitatively good flocculate. Said flocculate may become decanted and washed with demineralized water in order to remove the soluble salts and the development inhibiting crystal habit modifier e.g. adenine to an allowable residual amount (preferably at most 0.3 mg/g of gelatin) or applying an ultrafiltration washing procedure as disclosed e.g. in Research Disclosure, Vol. 102, Oct. 1972, Item 10208, Research Disclosure Vol. 131, March, Item 13122 and Mignot US-A 4,334,012. Said ultrafiltration technique may be applied on-line during the whole precipitation, in order to reduce the increasing amount of water, thus avoiding dilution of the reaction vessel and increasing amounts of soluble salts like the mainly occurring potassium nitrate. Examples thereof have been described e.g. in EP-A 0 577 886. When the emulsion after precipitation is washed by diafiltration by means of a semipermeable membrane, a technique also called ultrafiltration, it is not necessary to use polymeric flocculating agents that may disturb the coating composition stability before, during or after the coating procedure. Such procedures are disclosed e.g. in Research Disclosure Vol. 102, Oct. 1972, Item 10208, Research Disclosure Vol. 131, March, Item 13122 and US-P 4,334,012. Redispersion may further be performed by addition of extra hydrophilic colloid. As a consequence values of gesi and/or sisi may be enhanced up to values desired in order to prepare stable coating solutions. It is clear however that any useful protective colloid cited hereinbefore as an alternative of gelatin or gelatin in modified form may be used.

As already set forth additional gelatin or another hydrophilic colloid, suitable as a binder material can be added at a later stage of the emulsion preparation as e.g. after washing, in order to establish optimal coating conditions and/or to establish the required thickness of the coated emulsion layer. Preferably a gelatin to silver halide ratio, silver halide being expressed as an equivalent amount of silver nitrate, ranging from 0.3 to 1.0 is then obtained. Another binder may also be added instead of or in addition to gelatin. Useful vehicles, vehicle extenders, vehicle-like addenda and vehicle related addenda have been described e.g. in Research Disclosure N° 38957 (1996), Chapter II.

Prior to coating any thickening agent may be used in order to regulate the viscosity of the coating solution, provided that they do not particularly affect the photographic characteristics of the silver bromo iodide emulsion in the coated photographic material. Preferred thickening agents include aqueous polymers such as polystyrene sulphonic acid, dextran, sulphuric acid esters, polysaccharides, polymers having a sulphonic acid group, a carboxylic acid group or a phosphoric acid group as well as colloidal silica. Polymeric thickeners well-known from the literature resulting in thickening of the coating solution may even be used in combination with colloidal silica. Patents concerning thickening agents are e.g. US-A 3,167,410; Belgian Patent No. 558.143 and JP-A's 53-18687 and 58-36768. Negative effects on physical stability possibly resulting from the addition of polymeric compounds can be avoided by exclusion of those compounds and by restricting extra additions of colloidal silica. In order to coat hydrophilic colloidal layer compositions on a support by slide-hopper or curtain-coating techniques, wherein said compositions have gelatin in low amounts in order to provide a ratio by weight of gelatin to silver halide expressed as an equivalent amount of silver nitrate in the range from 0.05 to 0.4, thickening agents composed of synthetic clay and anionic macromolecular polyelectrolytes wherein said synthetic clay is present in an amount of at least 85 % by weight versus the total amount of thickening agents are recommended as has been disclosed in EP-A 0 813 105.

In order to reach a high hardening degree the layer binder should of course dispose of an acceptably high number of functional groups, which by reaction with an appropriate hardening agent can provide a sufficiently resistant layer. Such functional groups are especially the amino groups, but also carboxylic groups, hydroxy groups, and active methylene groups. Hardeners may be added to the antistress layer, covering one or more light-sensitive silver halide emulsion layers before or during the coating procedure, or to one or more of the said emulsion layers. The binders of the photographic element, especially when the binder used is gelatin, can be hardened with appropriate hardening agents such as those of the epoxide type, those of the ethylenimine type, those of the vinylsulfone type e.g. 1,3-vinylsulphonyl-2-propanol, chromium salts e.g. chromium acetate and chromium alum, aldehydes e.g. formaldehyde, glyoxal, and glutaraldehyde, N-methylol compounds e.g. dimethylolurea and methyloldimethylhydantoin, dioxan derivatives e.g. 2,3-dihydroxydioxan, active vinyl compounds e.g. 1,3,5-triacryloyl-hexa-hydro-s-triazine, active halogen compounds e.g. 2,4-dichloro-6-hydroxy-s-triazine, and mucohalogenic acids e.g. mucochloric acid and mucophenoxy-chloric acid. These hardeners can be used alone or in combination. The binders can also be hardened with fast-reacting hardeners such as carbamoylpyridinium salts. Formaldehyde and phloroglucinol can e.g. be added respectively to the protective layer(s) and to the emulsion layer(s). Preferred hardening agents in the context of the present invention however are bis-(vinylsulphonyl)-methane (BVSME) and ethylene bis-(vinyl-sulphone).

Direct X-ray materials according to the present invention, for use in the image-forming system according to the present invention, commonly have a hardening degree in order to have an absorption of water, as can be measured in a processing cycle after rinsing and before drying not, of not more than 2 g per g of gelatin coated.

A lot of other ingredients are further required in order get suitable sensitometric properties, as e.g. sensitivity (also called speed), gradation (also called contrast) and fog in the processing conditions for the materials coated from silver bromo iodide emulsions used in the element according to the present invention. Essentially the element according to the present invention is free from spectrally sensitizing dyes as those are playing no role in capturing direct X-rays.

Compounds preventing formation of fog or stabilizing the photographic characteristics during the production or storage of the photographic elements or during the photographic treatment thereof are required and are in most cases already present during emulsion precipitation and/or chemical sensitization. Many known compounds can be added as fog-inhibiting agent or stabilizer to the silver halide emulsion layer or to other coating layers in water-permeable relationship therewith such as an undercoat or a protective layer. Suitable examples are e.g. those described in Research Disclosure N° 17643 (1978), Chapter VI and in Research Disclosure N° 38957 (1996), Chapter VII.

The photographic element may further comprise various kinds of coating physical property modifying addenda as described in Research Disclosure N° 38957 (1996), Chapter IX, wherein coating aids, plasticizers and lubricants, antistats and matting agents have been described.

Development acceleration can be accomplished by incorporating in emulsion layer(s) or adjacent layers various compounds, preferably polyalkylene derivatives having a molecular weight of at least 400 such as those described in e.g. US-A's 3,038,805; 4,038,075 and 4,292,400 as well as in EP-A's 0 634 688 and 0 674 215.

The direct X-ray photographic element may further comprise various other additives such as e.g. compounds improving the dimensional stability of the photographic element, ultraviolet absorbers and spacing agents. Suitable additives for improving the dimensional stability of the photographic element are e.g. dispersions of a water-soluble or hardly soluble synthetic polymer e.g. polymers of alkyl(meth)acrylates, alkoxy(meth)acrylates, glycidyl (meth)acrylates, (meth)acrylamides, vinyl esters, acrylonitriles, olefins, and styrenes, or copolymers of the above with acrylic acids, methacrylic acids, α,β-unsaturated dicarboxylic acids, hydroxyalkyl (meth)acrylates, sulphoalkyl (meth)acrylates, and styrene sulphonic acids.

Suitable UV-absorbers are e.g. aryl-substituted benzotriazole compounds as described in US-A 3,533,794, 4-thiazolidone compounds as described in US-A 3,314,794 and 3,352,681, benzophenone compounds as described in JP-A 56-2784, cinnamic ester compounds as described in US-A's 3,705,805 and 3,707,375, butadiene compounds as described in US-A 4,045,229, and benzoxazole compounds as described in US-A 3,700,455 and those described in Research Disclosure N° 38957(1996), Chapter VI, wherein also suitable optical brighteners are mentioned.

Spacing agents may be present of which, in general, the average particle size is comprised between 0.2 and 10 µm. Spacing agents can be soluble or insoluble in alkali. Alkali-insoluble spacing agents usually remain permanently in the photographic element, whereas alkali-soluble spacing agents usually are removed therefrom in an alkaline processing bath. Suitable spacing agents can be made e.g. of polymethyl methacrylate, of copolymers of acrylic acid and methyl methacrylate, and of hydroxypropylmethyl cellulose hexahydrophthalate. Other suitable spacing agents have e.g. been described in US-A 4,614,708.

In direct X-ray photography the material has a duplitized emulsion layer coated on both sides (double-side coated) of the support. A mixture of two or more emulsions having silver bromo(chloro)iodide crystals with the same or different crystal sizes, the same or a different crystal habit, same or a different halide composition and/or a different or the same chemical ripening treatment, may be added to at least one light-sensitive emulsion layer, provided that at least one emulsion has crystals ripened with one or more selenium compounds as is essential in order to provide the material the tabular crystals with selenium in an amount of 0.5 to 20 µmole (and even more preferred 0.5 up to 10 µmole) per mole of silver nitrate.

Besides the light-sensitive emulsion layer(s) the photographic material may contain several light-insensitive layers at the side of the support carrying said light-sensitive emulsion layer(s), e.g. a protective antistress layer which can be split up into two layers, one of them being an underlying interlayer or an outermost afterlayer coated or sprayed on top of the "basic" protective antistress layer, one or more subbing layers, one or more intermediate layers, and even an afterlayer containing e.g. hardening agent(s), antistatic agent(s) and optionally filter dyes for safety-light purposes.

Protective antistress layers preferably contain coating aids and coating physical property modifying addenda mentioned in Research Disclosure No. 38957, published September 1996, Chapter IX. Antistatic properties are especially preferred in order to prevent blackening after processing in form of sparks, due to abrupt decharging of electrostatic charges during production and/or handling before exposure and/or processing. It is highly preferred to add antistatic agents to the protective antistress layer or to an afterlayer coated thereupon as has been described e.g. in EP-A's 0 534 006, 0 644 454 and 0 644 456 and in US-A's 4,670,374 and 4,670,376. In another embodiment antistatic agents as polythiophenes, or oxides of vanadium, tin, can also be added. Especially addition to the subbing layers of PEDT (a polythiophene) as described in EP 1 031 875 is recommended. Abrasion resistance of these outermost layers may be improved as described in US-A's 4,766,059 and 4,820,615. Spraycoating of afterlayers has been disclosed e.g. in US-A 5,443,640. Measures in order to further suppress pressure sensitivity may be coating of enhanced amounts of binder as e.g. gelatin. This however is disadvantageous with respect to rapid processing, especially drying, but measures as set forth in US-A 5,620,836 can also be applied in the present invention, offering however the particular advantage that less silver is coated in the elements according to the present invention as set forth hereinbefore. Moreover with respect to the binder material in the light-sensitive emulsion layer an improvement of pressure sensitivity can be expected if use is made therein from synthetic clays as has been disclosed in US-A 5,478,709.

In addition thereto it is recommended to prepare aqueous solid dispersions in colloidal silica for any photographically useful compound as has been suggested e.g. in EP-A 0 569 074. Advantages with respect to thin layer coating and rapid processing ability can be expected with relation thereto, without enhancing pressure sensitivity of more vulnerable layers.

The support of the direct X-ray radiographic elements of the present invention preferably is a blue colored polyester support like polyethylene terephthalate. The thickness of such organic resin film preferably is about 175 µm. Other suitable hydrophobic resin supports are well known to those skilled in the art and are made e.g. of polystyrene, polyvinyl chloride, polycarbonate and polyethylene naphthalate. The support is further provided with a substrate layer at both sides to have good adhesion properties between the adjacent layers and said support: one or more subbing layer(s) known to those skilled in the art for adhering thereto a hydrophilic colloid layer may be present. Suitable subbing layers for polyethylene terephthalate supports are described e.g. in US-A's 3,397,988, 3,649,336, 4,123,278 and 4,478,907. A preferred layer arrangement wherein a subbing layer composition comprising as a latex copolymer vinylidene chloride, methylacrylate and itaconic acid has been covered with hydrophilic layers being at least one gelatinous dye containing layer comprising one or more dyes, at least one silver halide emulsion layer, at least one protective antistress layer, and optionally an afterlayer has been described in EP-A 0 752 617. In that invention said hydrophilic layers have a swelling ratio of not more than 200 % and in said hydrophilic layers are coated simultaneously by the slide-hopper coating or by the slide-hopper curtain coating technique. Further information on suitable supports can be found in Research Disclosure No. 38957, Chapter XV, published September 1996.

According to the present invention a system for direct X-ray radiography comprised of (1) a direct X-ray radiographic element according to the present invention as set forth hereinbefore and 2) disposed on opposite sides of the direct X-ray element, two intensifying screens designed to emit electrons when exposed to X-or γ-rays with an energy greater than or equal to 10 kVp; more particularly with radiation having energies of 1.1 and 1.3 MeV as is the case for a Co-60 source or from a source for X-rays further comprising a high energy tube or even a synchrotron. High energy elementary particle radiation, generated from said high energy tube or from a synchrotron, as e.g. β-rays, electron beam or neutron radiation is useful in the context of the present invention.

According to the present invention a method is offered of providing an automated non-destructive test system to a manufacturing process, comprising the steps of providing at least one source for X-rays or γ-rays; and providing an object under test exposed to said X-rays or γ-rays, said object being operable to selectively absorb said X-rays or γ-rays.

In another embodiment according to the present invention a method is offered of providing a test system for personal monitoring as well as a personal electromagnetic radiation monitor wearable by person to warn the person of a radiation hazard condition caused by electromagnetic radiation emanating from a source of electromagnetic radiation, said monitor essentially comprising an element according to the present invention.

Further according to the present invention a method for forming a direct X-ray image, and more particularly, an industrial radiographic image for non-destructive testing purposes, has been provided, said method being comprised of (1) exposing the system disclosed hereinbefore to X- or γ-rays with an energy greater than or equal to 10 kVp to form a latent image and (2) developing (as part of a total processing cycle) the said latent image.

With respect to "ecological" processing methods, hardener-free black-and white developers are used, having ascorbic acid (as a more biodegradable developing agent instead of the conventional developing agents as dihydroxybenzene compounds or aminophenoles) as well as hardener-free fixers free from aluminum and/or ammonium salts, wherein said fixers further comprise a solvent for silver halides such as thiosulphate, thiocyanate or sulphurated organic compounds.

In a particularly preferred embodiment, according to the method of the present invention said latent image is developed in a developing bath which contains ascorbic acid as the developer. Information about such developers can be found e.g. in EP-A 0 732 619 and in US-A's 5,593,817; 5,604,082; 5,895,743 and 5,948,602; and in Research Disclosures Nos. 371052 (p. 185-224) and 352049 (p. 542-543), published March 1, 1995 and August 1, 1993 respectively.

In a further particularly preferred embodiment according to the method of the present invention said radiographic element is fully forehardened and the latent image is developed in a developing bath without further hardening. In practice this means that hydrophilic layers have a swelling ratio of not more than 200 %, more preferably not more than 150 %, and that in the processing cycle comprising the steps of developing, fixing, rinsing and drying, before drying and after the last rinsing step said material contains not more than 2 grams of water per gram of coated gelatin.

In one embodiment the image-forming method of the present invention comprises the step of processing said film material used in the image-forming system described hereinbefore, wherein said processing comprises the steps of developing in a developing solution comprising (iso)ascorbic acid, 1-ascorbic acid, reductic acid, salts and/or derivatives thereof; fixing in a fixer solution free from aluminum salts and, optionally, ammonium salts; rinsing and drying.

Replenishing said developing and fixer solution normally proceeds with amounts of replenisher in the range from 300 up to 900 ml/m², more preferably from 300 up to 600 ml/m², and from 400 up to 1200 ml/m², more preferably from 400 up to 700 ml/m², respectively. For the said processing, preferably an automatically operating apparatus is used provided with a system for automatic replenishment of the processing solutions. The processing therein proceeds within a relatively short processing time of from 1.5 up to 15 minutes from dry-to-dry, and more preferably and realistic, from 3 up to 8 minutes, for materials used in the image forming system of the present invention as with the radiographic element according to the invention, it is possible to use silver contents up to 25% lower than the silver contents of the emulsions with thick or three-dimensional grains of the elements for industrial radiography. A normally used configuration in the automatic processing apparatus shows the following consecutive tank units corresponding with, as consecutive solutions: developer-fixer-rinse water. In order to reduce "sludge formation" which is favored by solubilizing agents like sulphites, present in the developer as preservatives, a particularly suitable developer solution is the one comprising a reduced amount of sulphite and ascorbic acid which acts as a main developer and anti-oxidant as well and which is called "low-sludge" developer.

In favour of ecological fixation the presence of aluminum ions should be reduced, and more preferably, no aluminum ions should be present. This is moreover in favour of the absence of "sludge" formation, a phenomenon which leads to pi-line defects when high amounts of silver are coated in the light-sensitive layers. Measures in order to reduce "sludge-formation" have further been described in US-A's 5,447,817; 5,462,831 and 5,518,868. A particularly suitable fixer solution comprises an amount of less than 25 g of potassium sulphite per liter without the presence of acetic acid wherein said fixer has a pH value of at least 4.5, in order to make the fixer solution quasi odourless. The presence of α-ketocarboxylic acid compounds may be useful as has been described in EP-A's 0 620 483 and 0 726 491 and in Research Disclosure No. 16768, published March 1978. It is possible to use sodium thiosulphate as a fixing agent, thus avoiding the ecologically undesired ammonium ions normally used. For the relatively low coating amounts of silver halide as in the elements of the present invention a fixation time which is slightly reduced to about 100 seconds can be attained.

In another embodiment the developer solution used in the method according to this invention should be replenished not only for decrease of the liquid volume due to cross-over into the next processing solution but also for pH-changes due to oxidation of the developer molecules. This can be done on a regular time interval basis or on the basis of the amount of processed film or on a combination of both. In these circumstances, no dilution and mixing procedures are required before the regeneration bottles are adjusted to the processing unit. Moreover regeneration is kept to a minimum, especially in the processing of materials coated from lower amounts of emulsion crystals rich in silver bromide. Preferred minimum regeneration or replenishment amounts are from 300 up to 600 ml/m² for the developer solution and from 400 up to 700 ml/m² for the fixer solution. Replenishment of a developer comprising ascorbic acid or derivatives thereof and a 3-pyrazolidone derivative can be done as has been described in EP-A 0 573 700, wherein a method has been disclosed for processing with constant activity of image-wise exposed silver halide photographic material and wherein replenishing said developing solution proceeds by means of at least one replenishing solution having a higher pH than the developing solution. Other useful references related therewith, applicable with respect to the present invention, are e.g. EP-A's 0 552 511 and 0 660 175 and US-A's 5,503,965; 5,895,743 and 6,083,672.

The present invention is illustrated by the following examples, without however being limited thereto.

### COMPARATIVE EXAMPLES

### Example I.

The effect of chemical sensitization, making use of Se-compounds as sensitizers of AgBr(I) tabular grains or crystals having a thickness of the tabular grains of 0.22 µm will be illustrated hereinafter.

### Preparation of emulsion T, having tabular grains

To a solution of 5.5 g of oxidized gelatin (less than 30 µmole methionin per g) in 3 1 of demineralized water, adjusted to a pBr of 2.4 by adding KBr and a pH of 1.7 by adding H₂SO₄, were added by a double jet addition method aqueous solutions of 1.96 M AgNO₃ (hereinafter referred to as S1) and 1.96 M KBr (hereinafter referred to as S2) both at a constant flow rate of 16 ml/min during 27 seconds. During this period, the reaction mixture was maintained at 51°C. When the addition was completed, stirring continued during 1.5 minutes and then, temperature was increased up to 70°C over a period of 25 minutes, followed by addition of a NaOH solution over a period of one minute in order to adjust pH to a value of 5.6. Then stirring continued for 2.5 minutes and 0.5 1 of a 10 % gelatin solution, kept at 70°C, was added. After stirring during another 5.5 minutes, S2 was added in a single jet at 7.5 ml/min over a period of 5.5 minutes. Then S1 at a constant flow rate of 7.5 ml/min and S2 at a flow rate, controlled in order to maintain pAg at 8.9, were added by double jet addition over a period of 1 minute. This double jet was continued during another period of 33 minutes and 23 seconds, while the flow rate of S1 was linearly increased up to 23.1 ml/min and pAg was maintained at 8.9. 5 minutes after the completion of said double jet addition, S1 was added at 7.5 ml/min during 7 minutes and 20 seconds. Then another double jet started of S1 at 7.5 ml/min during 1 minute and 40 seconds and an aqueous solution of 1.93 M KBr and 0.03 M KI at a controlled flow rate in order to maintain pAg at 7.4. This double jet was continued during another period of 40 minutes and 56 seconds, while the flow rate of S1 was linearly increased up to 36.8 ml/min and pAg was maintained at 7.4. The average grain size, derived from electron microscopic photographs and calculated as average equivalent circular diameter of the corresponding tabular grains of the emulsion thus prepared was 0.78 µm, the average thickness was 0.22 µm and the variation coefficient was 0.30. The iodide content was 1 mole % based on silver. After washing, gelatin and water were added in order to obtain a silver halide content of 245 g/kg, expressed as AgNO₃, and a gelatin content of 83 g/kg. The pH was adjusted to 6.0.

### Chemical ripening:

Per mole of AgBr(I) following addenda were consecutively furnished, providing a time of 10 minutes between their addition:
- sodium thiosulphate (in an amount as indicated in Table 1)
- selenium compound (in an amount as indicated in Table 1, structures as indicated hereinafter) Both compounds I and II were dissolved in methanol solution in a concentration of 1 g/l.
- 18 ml of a water solution containing 1.46x10⁻³ M chloroauric acid and 1.58x10⁻² M ammonium thiocyanate.
- 13ml of a water solution containing 7,93x10⁻³ M Na₂SO₃.

The emulsions were heated for 4 hours at 52°C.

After cooling, a preservative was added.

### Coating of the emulsion (see Table 1):

Compounds added to the silver bromoiodide emulsion, in grams per mole of equivalent amounts of AgNO₃.

### Composition of the top-coating (protective antistress layer) in g per m² after coating (see Table 2)

**Table 2**

| Compound | Amount in g/m2 |
|---|---|
| Gelatin | 1.89 |
| Polymethylmethacrylate spacing agent (average particle diameter 3 mm) | 0.011 |
| Chromium acetate | 0.0077 |
| CF₃- (CF₂)₆-COOH.NH3 | 0.0074 |
| CF₃-(CF₂)₆-CONH- (CH₂CH₂O)₁₇₋₂₀-H: | 0.020 |
| Mobilcer Q (a paraffin wax, trade name product from MOBIL OIL) | 0.023 |
| Polythioether A (modified poly-epichlorohydrine having an average chain length of approximately 20 monomer units and of which about 50% of the chloride groups have been replaced by a -S-CH₂-CHOH-CH₂OH substituent) | 0.042 |
| Bis-vinyl-sulphonyl-methyl ether (added just | 0.130 |
| (before coating) | |

### Coating of the materials

The photographic materials according to these examples comprise one emulsion layer and one protective layer, coated symmetrically in the same way at both sides of a blue colored polyethylene terephthalate support having a density for white light of 0.150 and a thickness of 175 µm. The coating solution of the emulsion layer was prepared by adding solutions of the compounds indicated in Table 1 to the emulsions dissolved while heating and stirring. The coating solution of the protective layer has been given in Table 2.
After adjusting the pH to 6.8, the viscosity and surface tension of the coating solutions were optimized according to the requirements of the coating method.
The emulsion layer and the protective layer were coated simultaneously on one side of the subbed polyester support, mentioned hereinbefore by means of the conventional slide hopper coating techniques. The silver coverage of the emulsions was 11.5g/m², expressed as equivalent amount of AgNO₃/m² per side.

### Exposure conditions, processing conditions and determination of sensitometric parameters.

Samples of said coated and dried films were
(1) exposed according to ISO7004 with a 220kV radiation source with a copper filter of 8 mm thickness and
(2) exposed with a Co-60 radiation source.

The exposed samples were developed, fixed, rinsed and dried in an automatic processing machine, called Stucturix NDT-S, marketed by Agfa-Gevaert. The processing cycle was 8 minutes, the developer temperature was 28°C. Developer and fixer solutions were the commercially available Agfa-Gevaert NDT G135 and G335 respectively.

After processing the following sensitometric parameters were determined:
(i) Dₘᵢₙ : optical density in thousands of log units of a non-exposed sample including the density of the blue colored polyester layer layer;
(ii) Speed : measured as the log E value at a density of Dmin + 2.0 (a lower figure is representative for a higher speed).
(iii) Relative speed: a commercially available Agfa-Gevaert Structurix D7 film (emulsion number 4370041) was exposed, processed and measured under equal conditions as the above mentioned samples. The relative speed was calculated as the difference in logE between the speed of the sample and the Structurix D7 film, taken as a reference sample. A positive figure is thus indicative for a more sensitive sample than the Structurix D7 reference.

The said Structurix® D7 film contains cubic silver bromoiodide emulsion crystals having an average grain size of 0.54 µm.

The results, summarized in Table 3 hereinafter, clearly show that the addition of compound I results in a significant increase of sensitivity for radiation from the 220kV X-ray source and even in a much higher sensitivity gain for high energy radiation from a Co⁶⁰ source. With the addition of comound I it is possible to obtain an equal sensitivity difference with the reference sensitivity for both radiation sources.

The remarkably high gain in sensitivity for Co-60 radiation was completely unexpected.

**Table 3**

| Sodium thiosulphate µmole/mole of Ag | Se compound I µmole/mole of Ag | Dₘᵢₙ | 220kV speed | 220kV speed relative | Co-60 Speed | Co-60 Speed Relative |
|---|---|---|---|---|---|---|
| Structurix D7 4370041 | | 200 | 0.153 | 0 | 3.53 | 0 |
| 2.70 | 0 | 157 | 0.147 | +0.006 | 3.63 | -0.010 |
| 2.70 | 2.60 | 174 | 0.132 | +0.021 | 3.30 | +0.023 |
| 2.70 | 5.20 | 175 | 0.123 | +0.030 | 3.16 | +0.037 |
| 6.70 | 0 | 160 | 0.140 | +0.013 | 3.49 | +0.005 |
| 6.70 | 2.60 | 167 | 0.125 | +0.028 | 3.26 | +0.027 |
| 6.70 | 5.20 | 179 | 0.122 | +0.031 | 3.17 | +0.037 |
| 10.80 | 0 | 164 | 0.137 | +0.016 | 3.45 | +0.008 |
| 10.80 | 2.60 | 162 | 0.124 | +0.029 | 3.19 | +0.034 |
| 10.80 | 5.20 | 160 | 0.125 | +0.028 | 3.20 | +0.033 |

### Example II.

The experimental conditions in the present Example are the same as in Example I, except for use of compound II as a source of selenium in the chemical sensitization step. The results thus obtained have been summarized in Table 4.

**Table 4**

| Sodium thiosulphate µmole/mole of Ag | Se compound II µmole/mole of Ag | Dₘᵢₙ | 220kV speed | 220kV speed relative | Co-60 Speed | Co-60 Speed Relative |
|---|---|---|---|---|---|---|
| Structurix D7 4370041 | | 190 | 1.51 | 0.00 | 3.50 | 0.00 |
| 2.70 | 0 | 151 | 1.45 | +0.06 | 3.59 | -0,09 |
| 2.70 | 3.10 | 166 | 1.30 | +0.21 | 3.29 | +0.21 |
| 6.70 | 0 | 150 | 1.39 | +0.12 | 3.46 | +0.04 |
| 6.70 | 3.10 | 173 | 1.29 | +0.22 | 3.26 | +0.24 |
| 10.80 | 0 | 153 | 1.36 | +0.15 | 3.43 | +0.07 |
| 10.80 | 3.10 | 159 | 1.28 | +0.23 | 3.20 | +0.30 |

Fully in accordance with the results obtained in the previous Example I, addition of a selenium compound in the chemical ripening again results in a significant increase in sensitivity, more particularly when exposing the materials with the high energy radiation of a Co-60 source.

### Example III.

In this example the effect of chemical sensitization when adding a selenium compound in the chemical sensitizing step on thin tabular grains (having a thickness of 0.12 µm) has been shown.

### Preparation of the tabular AgBr(I) emulsion T'.

To a solution of 6.9 g of an oxidized gelatin in 3 1 of demineralized water at 51°C, adjusted to a pH of 2.5 by adding H2SO4, stirred up to a rate of 600 r.p.m., were added by a double jet method aqueous solutions of 0.98 M AgNO3 (hereinafter referred to as A1) and 0.98 M KBr (hereinafter referred to as B1) : 25 ml of A1 and 25 ml of B1 were added in a time interval of 30 seconds. When the addition was completed, the temperature was increased up to 70°C over a period of 30 minutes: UAg was controlled (expressed in mV versus a Ag/AgCl(sat.) reference electrode and should be in the range from 44.5 + 5 mV at a temperature of 70°C + 1°C. 1 minute later pH was set to a value of 5.0 + 0.3 and immediately thereafter a solution of 50 g of inert gelatin in 500 ml of demineralized water of 70°C was added. 3 minutes later B1 was added at a rate of 7.06 ml/min. during 120 seconds, while simultaneously adding by double jet A1 at a rate of 7.5 ml/min.). In a further double jet addition A1 and B1 were added during 2822 seconds at a linearly increasing rate going from 7.0 up to 21.11 ml/min. for A1 and from 7.06 up to 21.29 ml/min for 81 in order to maintain a constant UAg potential of + 40 mV in the reaction vessel. After 5 minutes A1 and B1 were simultaneously added by double-jet addition during 60 seconds at a rate of 10.0 and 10.04 ml/min. respectively whereby the UAg value was held at a constant value of 50 mV while increasing the flow rate up to 46.49 ml/min. and 46.69 ml/min. respectively over a total time period of 81 min. and 5 seconds.

After that double-jet addition period, an amount of an emulsion having ultrafine (ca. 0.040 µm) 100 % AgI crystals, dissolved in 20 g of demineralized water at 40°C, was added to the reaction vessel in order to get a total AgI content at the end of precipitation of 0.1 mole % vs. silver precipitated.

The average grain size of the silver bromoioide tabular {111} emulsion grains thus prepared, expressed as equivalent volume diameter, was 0.53 µm, the average thickness was 0.09 µm.

After washing, gelatin and water were added in order to obtain a silver halide content of 245 g/kg, expressed as AgNO₃/m², and a gelatin content of 83 g/kg. The pH was adjusted to 6.0.

The following part of the experimental procedure was equal to the procedure described in Example I, except for the Ag content of the coated samples which was 20 g/m2, expressed as AgNO₃ as before.

Results of this experiment have been summarized in the same way as before, in Table 5.

**Table 5.**

| Sodium thiosulphate µmole/mole of Ag | Se-compound I µmole/mole of Ag | Dₘᵢₙ | 220kV speed | 220kV speed relative | Co-60 Speed | Co-60 Speed Relative |
|---|---|---|---|---|---|---|
| Structurix D7 4370041 | | 200 | 1.54 | 0 | 3.54 | 0 |
| 6.70 | 0 | 155 | 1.43 | +0.11 | 3.61 | -0.07 |
| 6.70 | 2.50 | 159 | 1.14 | +0.40 | 3.10 | +0.44 |
| 6.70 | 5.00 | 162 | 1.10 | +0.44 | 3.01 | +0.53 |

The results in Table 5 show that even for thin tabular grains addition of compound I results in a clear increase of sensitivity for radiation from the 220kV X-ray source and in a higher sensitivity gain for high energy radiation from a Co-60 source.

Having described in detail preferred embodiments of the current invention, it will now be apparent to those skilled in the art that numerous modifications can be made therein without departing from the scope of the invention as defined in the appending claims.

## Claims

1. Direct X-ray radiographic element comprised of a support covered on at least one of its major faces with a tabular grain emulsion layer free from spectrally sensitizing dyes, in which at least 50 percent of total grain projected area is accounted for by silver bromoiodide tabular grains having silver iodide in an amount of at most 1 mole % based on silver, having an average volume between 0.05 and 2 µm³ and an average aspect ratio between 5 and 25, wherein a silver content per coated side, expressed as an equivalent amount of silver nitrate, is between 5 and 25 g/m², **characterized in that** said tabular grain emulsion(s) have selenium in an amount of 0.5 to 20 µmole per mole of silver nitrate.

2. System for direct X-ray radiography comprised of
(1) a direct X-ray radiographic element according to claim 1 and
(2) disposed on opposite sides of the said element, two intensifying screens designed to emit electrons when exposed to X or gamma rays with an energy greater than or equal to 10 kVp.

3. System according to claim 2, wherein said energy is corresponding with the energy of a Co-60 source having radiation energies of 1.1 and 1.3 MeV.

4. System according to claim 2 or 3, wherein said intensifying screens are screen sheets selected from the group consisting of lead, lead oxide, copper and steel.

5. Method of forming a radiographic image comprised of
(1) exposing a system according to claim 2, to X- or γ-rays with an energy greater than or equal to 10 kVp in order to form a latent image and (2) developing said latent image.

6. Method of forming a radiographic image comprised of
(1) exposing a system according to claim 3, with the energy of a Co-60 source in order to form a latent image and
(2) developing said latent image.

7. Method according to claim 6, wherein said latent image is developed in a developing bath which contains ascorbic acid as a developing agent.

8. Method according to claim 6 or 7, wherein said radiographic element is fully forehardened and wherein the latent image is developed in a developing bath without further hardening.

9. A personal electromagnetic radiation monitor wearable by a person to warn the person of a radiation hazard condition caused by electromagnetic radiation emanating from a source of electromagnetic radiation, said monitor essentially comprising an element according to claim 1.

10. Element according to claim 1, wherein said element is an industrial non-destructive testing material.

## Patentansprüche

1. Ein gegenüber direkter Röntgenstrahlung empfindliches radiografisches Element mit einem Träger, der auf zumindest einer Hauptfläche mit einer tafelkörnigen, keine spektralsensibilisierenden Farbstoffe enthaltenden Emulsion beschichtet ist, wobei zumindest 50% der gesamten, mit Körnern beschichteten Oberfläche aus tafelförmigen Silberbromidiodidkörnern mit einem Silberiodidgehalt von höchstens 1 mol-%, bezogen auf den Silbergehalt, besteht, wobei die Silberiodidkörner ein mittleres Volumen zwischen 0,05 und 2 *µ*m³ und ein mittleres Aspektverhältnis zwischen 5 und 25 aufweisen und der als äquivalente Menge Silbernitrat ausgedrückte Silbergehalt pro emulsionierte Seite zwischen 5 und 25 g/m² liegt, **dadurch gekennzeichnet, dass** die tafelkörnige(n) Emulsion(en) Selen in einer Menge von 0,5 bis 20 *µ*Mol pro Mol Silbernitrat enthält (enthalten).

2. Direktes Röntgensystem enthaltend :
(1) ein direktes Röntgenelement nach Anspruch 1 und
(2) auf gegenüberliegenden Seiten des radiografischen Elements zwei Verstärkerfolien, die bei Belichtung mit Röntgenstrahlung oder Gammastrahlung mit einer Intensität von zumindest 10 kVp Elektronen emittieren.

3. System nach Anspruch 2, **dadurch gekennzeichnet, dass** die Energie der Energie einer Co-60-Quelle mit einer Strahlungsenergie zwischen 1,1 und 1,3 MeV entspricht.

4. System nach Anspruch 2 oder 3, **dadurch gekennzeichnet, dass** die Verstärkerfolien Folienblätter aus der Gruppe bestehend aus einer Bleifolie, einer Bleioxidfolie, einer Kupferfolie und einer Stahlfolie sind.

5. Ein durch die nachstehenden Schritte **gekennzeichnetes** Verfahren zur Erzeugung eines Röntgenbildes :
(1) Belichtung eines Systems nach Anspruch 2 mit entweder Röntgenstrahlung oder Gammastrahlung mit einer Intensität von zumindest 10 kVp zur Erzeugung eines latenten Bildes und
(2) Entwicklung des latenten Bildes.

6. Ein durch die nachstehenden Schritte **gekennzeichnetes** Verfahren zur Erzeugung eines Röntgenbildes :
(1) Belichtung eines Systems nach Anspruch 3 mit der Energie einer Co-60-Quelle zur Erzeugung eines latenten Bildes und
(2) Entwicklung des latenten Bildes.

7. Verfahren nach Anspruch 6, **dadurch gekennzeichnet, dass** das latente Bild in einem Ascorbinsäure als Entwicklersubstanz enthaltenden Entwicklerbad entwickelt wird.

8. Verfahren nach Anspruch 6 oder 7, **dadurch gekennzeichnet, dass** das Röntgenelement völlig vorgehärtet ist und das latente Bild ohne weitere Härtung in einem Entwicklerbad entwickelt wird.

9. Ein persönlicher elektromagnetischer Strahlungsmelder, der von einer Person getragen werden kann und die Person vor Bedingungen mit Strahlungsgefahr warnt, denen von einer elektromagnetischen Strahlungsquelle herrührende elektromagnetische Strahlung zugrunde liegt, wobei der Melder im wesentlichen aus einem Element nach Anspruch 1 aufgebaut ist.

10. Element nach Anspruch 1, **dadurch gekennzeichnet, dass** das Element ein Material für industrielle zerstörungsfreie Prüfungen ist.

## Revendications

1. Élément pour la radiographie directe par rayons X comprenant un support recouvert, sur au moins une de ses faces majeures, d'une couche d'émulsion à grains tabulaires exempte de colorants sensibilisateurs spectraux, dans lequel au moins 50 % de la surface projetée des grains totale est occupée par des grains tabulaires au bromoiodure d'argent possédant une teneur maximale en iodure d'argent s'élevant à 1 mole %, basé sur la teneur en argent, possédant un volume moyen entre 0,05 et 2 µm³ et un rapport nominal d'aspect moyen entre 5 et 25, dans lequel la teneur en argent par côté muni d'un revêtement, exprimée comme quantité équivalente de nitrate d'argent, se situe entre 5 et 25 g/m², **caractérisé en ce que** ladite ou lesdites émulsions à grains tabulaires possèdent du sélénium en une quantité de 0,5 à 20 *µ*m par mole de nitrate d'argent.

2. Système pour la radiographie directe par rayons X comprenant : (1) un élément pour la radiographie directe par rayons X selon la revendication 1 et : (2), disposés sur les côtés opposés dudit élément, deux écrans renforçateurs conçus pour émettre des électrons lors d'une exposition à des rayons X ou à des rayons gamma, possédant une énergie supérieure ou égale à 10 kVp.

3. Système selon la revendication 2, dans lequel ladite énergie correspond à l'énergie d'une source de cobalt 60 possédant des énergies de rayonnement de 1,1 et de 1,3 MeV.

4. Système selon la revendication 2 ou 3, dans lequel lesdits écrans renforçateurs sont des feuilles faisant office d'écrans choisis parmi le groupe constitué par le plomb, l'oxyde de plomb, le cuivre et l'acier.

5. Procédé pour la formation d'une image radiographique comprenant le fait de (1) exposer un système selon la revendication 2 à des rayons X ou à des rayons gamma possédant une énergie supérieure ou égale à 10 kVp pour former une image latente et (2) développer ledit image latente.

6. Procédé pour la formation d'une image radiographique comprenant le fait de (1) exposer un système selon la revendication 3, avec l'énergie d'une source de colbalt 60 pour former une image latente et (2) développer ladite image latente.

7. Procédé selon la revendication 6, dans lequel ladite image latente est développée dans un bain de développement qui contient de l'acide ascorbique à titre d'agent développateur.

8. Procédé selon la revendication 6 ou 7, dans lequel ledit élément radiographique est soumis à un durcissement complet préalable et dans lequel l'image latente est développée dans un bain de développement en l'absence d'un durcissement ultérieur.

9. Moniteur personnel de rayonnements électromagnétiques qui peut être porté par une personne pour avertir la personne d'un état de risque de rayonnement provoqué par un rayonnement électromagnétique émanant d'une source de rayonnements électromagnétiques, ledit moniteur comprenant essentiellement un élément selon la revendication 1.

10. Élément selon la revendication 1, dans lequel ledit élément est un matériau d'essai non destructif à l'échelle industrielle.
